

# UNITED STATES PATENT OFFICE.

KARL ARNOLD, OF NUREMBERG, GERMANY.

## PROCESS OF MAKING A FRICTION IGNITER.

1,404,261.

Specification of Letters Patent. Patented Jan. 24, 1922.

No Drawing.

Application filed July 14, 1921. Serial No. 484,836.

To all whom it may concern:

Be it known that I, KARL ARNOLD, a citizen of the German Empire, residing at Blumenthalstrasse 4, Nuremberg, Bavaria, 5 Germany, have invented a new and useful Process of Making a Friction Igniter, (for which I have filed an application in Germany, July 8, 1919,) of which the following is a specification.

10 My invention relates to a process of making a friction-igniter to be used as a substitute for cerium iron alloy and the object of my invention is to provide for a device or substance doing the same service with equal 15 efficiency as the material named and being particularly adapted for use in connection with toys.

Another advantage of my invention is that the product to which it refers has 20 shown itself as air-proof and durable while cerium iron alloy is liable to decay and disintegration. The formation of sparks is

with the product of my invention in no way smaller than is the case with cerium iron alloy.

25

The process consists of applying the waste of powdered pyrophorous metal or alloy, as, for instance, cerium alloy on paper or paper fabric or other suitable support of various strengths by means of any suitable 30 agglutinant.

I claim:—

1. The herein described process of making a friction-igniter consisting of applying the powdered waste of pyrophorous metal or 35 alloy on paper or paper fabric by means of an agglutinant.

2. A match consisting of the powdered waste of pyrophorous metal or alloy secured to a support of paper or paper fabric by 40 means of an agglutinant.

In testimony whereof I affix my signature.

KARL ARNOLD.